

1

3,371,042

## FERROMAGNETIC MATERIALS

Thomas R. McGuire and Merrill W. Shafer, Yorktown Heights, N.Y., assignors to International Business Machines Corporation, New York, N.Y., a corporation of New York  
 No Drawing. Filed Jan. 28, 1965, Ser. No. 428,862  
 8 Claims. (Cl. 252—62.51)

## ABSTRACT OF THE DISCLOSURE

Ferromagnetic compositions represented by the formula  $(\text{EuO})_{1-x}(\text{RS})_x$  in which  $0.01 < x < 0.30$  and R is a rare earth. The compositions are characterized by a Curie temperature which can be controlled between 73° K. and 132° K.

This invention relates to a new series of europium compounds exhibiting a paramagnetic Curie temperature ( $\theta$ ) which can be selectively varied between 73° K. and 132° K. In accordance with this invention, the paramagnetic Curie temperature ( $\theta$ ) of such compounds is varied by changing the population of electrons in the d-orbitals of the base europium oxide (EuO) material while retaining the characteristically high magnetic moment thereof.

With the discovery of ferromagnetism in the europium chalcogenide series, a new group of materials with device applications has become available. One such material is europium oxide (EuO) which exhibits desirable characteristics, i.e., high magnetic moment; however, europium oxide (EuO) exhibits a relatively low paramagnetic Curie temperature ( $\theta$ ) of 73° K. Paramagnetic Curie temperature ( $\theta$ ) is a measure of the ferromagnetic exchange interactions and is closely related to the Curie temperature where spontaneous magnetization occurs. Accordingly, present use of europium oxide for device applications is seriously limited since devices formed thereof cannot be operated at convenient temperatures, say liquid nitrogen ( $\text{N}_2$ ) temperatures (77° K.). The usefulness of europium oxide (EuO) would be obviously increased if the respective paramagnetic Curie temperature ( $\theta$ ) exhibited thereby could be raised at least above the temperature of liquid nitrogen ( $\text{N}_2$ ) at atmospheric pressures.

The ferromagnetic saturation moment of europium oxide (EuO) is higher than those of ferrites which, for example, have saturation moments below 6,000 gauss. Therefore, europium oxide (EuO) would provide a useful magnetic material for application where high magnetic moments are desired (high frequency transformer cores, microwave gyrators, etc.).

Generally, the structure of europium oxide (EuO) can be characterized as having a half-filled 4f shell and an empty 5d shell. Paramagnetic Curie temperature ( $\theta$ ) is affected by changing the population of electrons in the europium oxide (EuO) to vary electron concentrations in the crystal lattice. According to molecular field theory, magnetic interactions between electron spin moments is determinative of the paramagnetic Curie temperature ( $\theta$ ). The interaction between magnetic spin moments which produces spontaneous magnetization in europium oxide (EuO) has been explained by the interaction between spin moments of the nearest neighbor europium (Eu) ions in the rock salt-type face centered cubic crystal structure of europium oxide (EuO). Reference is made to patent application Ser. No. 374,351, filed June 11, 1964, in the names of F. Holtzberg et al., entitled "New Ferromagnetic Materials," and assigned to the assignee of this invention. Since the electron spin moments of the 4f and 5d shells of neighboring europium ions ( $\text{Eu}^{++}$ )

2

overlap, there is a virtual occupation of the 5d shell which gives rise to exchange interactions. The virtual occupation of the 5d shell would allow the filling of the  $t_{2g}$  orbitals which would overlap in the (110) direction and effectively increase magnetic interactions between neighboring europium ions ( $\text{Eu}^{++}$ ) whereby the paramagnetic Curie temperature ( $\theta$ ) is increased. The amount of increase in paramagnetic Curie temperature ( $\theta$ ) varies as the increased electron concentration in the crystal lattice of the europium oxide (EuO).

In accordance with this invention, the paramagnetic Curie temperature ( $\theta$ ) of europium oxide (EuO) is adjusted by forming a solid solution having the formula  $(\text{EuO})_{1-x}(\text{RS})_x$ , where  $0.01 < x < 0.30$ , (RS) is a monosulfide, and (R) is a rare earth selected from the group consisting of lanthanum (La), praseodymium (Pr), neodymium (Nd), samarium (Sm), gadolinium (Gd), cerium (Ce), dysprosium (Dy), terbium (Tb), holmium (Ho), erbium (Er), thulium (Tm), and lutetium (Lu). In accordance with this invention, albeit a two-phase system may result, the solid solution of the monosulfide (RS) in europium oxide (EuO) exhibits a substantial increase in paramagnetic temperature ( $\theta$ ).

It is an object of this invention to provide a new series of europium compounds exhibiting a Curie temperature ( $\theta$ ) which can be controlled between 73° K. and 132° K.

Another object of this invention is to prepare a material exhibiting a relatively high magnetic moment and having a paramagnetic Curie temperature ( $\theta$ ) in excess of liquid nitrogen ( $\text{N}_2$ ) temperatures (77° K.).

Another object of this invention is to provide a process for controlling the Curie temperature ( $\theta$ ) of magnetic materials formed of europium oxide (EuO).

Another object of this invention is to provide a ferromagnetic material having the formula  $(\text{EuO})_{1-x}(\text{RS})_x$ , where  $0.01 < x < 0.30$ .

The novel ferromagnetic material of this invention is prepared by homogeneously mixing appropriate predetermined quantities of the base europium oxide (EuO) and monosulfide material (RS), where (RS) is a monosulfide and (R) is a rare earth selected from the group consisting of lanthanum (La), praseodymium (Pr), neodymium (Nd), samarium (Sm), gadolinium (Gd), cerium (Ce), dysprosium (Dy), terbium (Tb), holmium (Ho), erbium (Er), thulium (Tm), and lutetium (Lu). The europium oxide (EuO) and monosulfide (RS), thus mixed, are heated to a reaction temperature at least lower than the decomposition temperature of either material and then cooled rapidly to room temperature. The quantity of monosulfide material (RS) added to the base europium oxide (EuO) material is determinative of the change in paramagnetic Curie temperature ( $\theta$ ) of the reacted mixture, i.e., of the europium oxide (EuO). The reacted mixture may define at least a two-phase system, one such phase being a solid solution monosulfide of the (RS) and europium oxide (EuO).

This procedure involved in forming the novel ferromagnetic material of this invention is to initially blend, e.g., by mechanical shaker, mortar and pestle, etc., appropriate amounts of the base europium oxide (EuO) material and the modifying monosulfide material (RS), each in finely divided form, to obtain a homogeneous mixture. The homogeneous mixture of the base europium oxide (EuO) material and the monosulfide material (RS) are pressed into pellets, e.g., by a hydraulic press, and then heated to between 1500° C. and 1950° C. in a nonoxidizing atmosphere. For example, the pellets may be heated in a refractory metal crucible, e.g., molybdenum, tantalum, etc., which is evacuated and sealed. Alternatively, the mixture can be placed in an open crucible and heated in a reducing atmosphere, e.g., helium, argon, etc. In either event, the pellets are heated in the described temperature

range in excess of one hour so as to insure reaction of the base europium oxide (EuO) material and the monosulfide material (RS) to support the formation of a solid solution. Best results have been observed when the monosulfide (RS)-europium oxide (EuO) mixture is heated sufficiently to cause a portion of the mixture to pass into the liquid phase and rapidly cool to room temperature, for example, within 30 minutes. The reacted mixture, when cooled, retains the desired magnetic properties of europium oxide (EuO) but exhibits a paramagnetic Curie temperature ( $\theta$ ) which can be adjusted to exceed liquid nitrogen ( $N_2$ ) temperatures.

The paramagnetic Curie temperature ( $\theta$ ) is increased due to the introduction of additional electrons into the rock-salt structure of the base europium oxide (EuO) material by the monosulfide (RS) whereby the electron concentration of the former is increased. Since the (R) constituent, above identified, of the monosulfide (RS) material is trivalent, it can be theorized that the substitution of trivalent ( $R^{+++}$ ) ions for the ( $Eu^{++}$ ) ions in the lattice introduced electrons into the  $5d$  shell of remaining ( $Eu^{++}$ ) ions in the lattice. Due to the presence of the trivalent ( $R^{+++}$ ) ions, the  $5d$  shells of the remaining ( $Eu^{++}$ ) ions are virtually occupied and magnetically coupled in the (110) direction so as to increase magnetic interaction between adjacent ( $Eu^{++}$ ) ions in the lattice. The resulting virtual occupation of the  $5d$  shells ( $t_{2g}$ ) gives rise to exchange interactions effective to increase the paramagnetic Curie temperature ( $\theta$ ) in excess of liquid nitrogen ( $N_2$ ) temperature ( $77^\circ K.$ ).

#### Example 1

Ferromagnetic materials of this invention have been prepared in accordance with the following table where the following percentages in moles of europium oxide (EuO) and cerium sulfide (CeS) were reacted to obtain the indicated paramagnetic Curie temperature ( $\theta$ ).

TABLE I

| EuO (moles) | CeS (moles) | Paramagnetic Curie temperature ( $\theta$ ), $^\circ K.$ |
|-------------|-------------|----------------------------------------------------------|
| 98          | 2           | 73                                                       |
| 95          | 5           | 78                                                       |
| 92          | 8           | 85                                                       |
| 85          | 15          | 130                                                      |
| 80          | 20          | 132                                                      |
| 70          | 30          | 130                                                      |

The europium oxide (EuO) and cerium sulfide (CeS) materials in finely powdered form in the amounts shown in Table I were mixed by mortar and pestle to obtain a homogeneous mixture. The homogeneous mixture was pressed into pellets and placed in an open tantalum crucible. The tantalum crucible was heated in an argon (Ar) atmosphere for approximately 8 hours at  $1700^\circ C.$ , a portion of the mixture being observed to pass into the liquid phase, and cooled down to room temperature within a 30-minute period. The reacted mixtures each formed a two-phase system and exhibited increased paramagnetic Curie temperature ( $\theta$ ) which varied as the percentage by mole of the modifying cerium sulfide (CeS) material, as shown in Table I. Part of the reacted material had a rock-salt structure. When the percentage by mole of cerium sulfide (CeS) was increased to 5 percent, the reacted mixture exhibited ferromagnetic properties at  $78^\circ K.$  or above liquid nitrogen ( $N_2$ ) temperatures. Also, the reacted mixture exhibited increased electrical conductivity as the percentage by mole of cerium sulfide (CeS) was increased. The observed paramagnetic Curie temperature ( $\theta$ ) of  $130^\circ K.$  when 70 percent by mole of europium oxide (EuO) was reacted with 30 percent by mole of cerium sulfide (CeS) was within experimental error.

#### Example 2

Also, similar procedures have been employed to prepare ferromagnetic materials of this invention wherein the fol-

lowing percentages by mole of europium oxide (EuO) and lanthanum sulfide (LaS) as shown in the Table II were reacted to obtain the indicated paramagnetic Curie temperatures ( $\theta$ ).

TABLE II

|    | EuO (moles) | LaS (moles) | Paramagnetic Curie temperature ( $\theta$ ), $^\circ K.$ |
|----|-------------|-------------|----------------------------------------------------------|
| 10 | 99          | 1           | 73                                                       |
|    | 95          | 5           | 80                                                       |
|    | 90          | 10          | 90                                                       |
|    | 89          | 20          | 100                                                      |
|    | 70          | 30          | 130                                                      |

Finely-powdered europium oxide (EuO) and lanthanum sulfide (LaS) materials were homogeneously mixed by mortar and pestle and pressed into pellets. The pellets were placed into an open tantalum crucible and heated at  $1750^\circ C.$  in a nitrogen ( $N_2$ ) atmosphere for approximately 8 hours and then cooled to room temperature within a 30-minute period. During the heat treatment, a portion of the mixture was observed to pass into the liquid phase. As the percentage by mole of lanthanum sulfide (LaS) was increased, the paramagnetic Curie temperature ( $\theta$ ) of the reacted mixture rose as indicated in Table II. The presence of 5 percent by mole of lanthanum sulfide (LaS) was effective to increase the paramagnetic Curie temperature ( $\theta$ ) of the reacted mixture to approximately  $80^\circ K.$ , i.e., in excess of liquid nitrogen ( $N_2$ ) temperatures. Also, the reacted mixtures each formed a two-phase system and exhibited increased electrical conductivity as the percentage by mole of lanthanum sulfide (LaS) was increased.

#### Example 3

Similar procedures were followed as in Examples 1 and 2 with respect to the europium oxide (EuO)-erbium sulfide (ErS) series. Fifteen percent by mole of erbium sulfide (ErS) was reacted with 85 percent by mole of europium oxide (EuO). Again, finely-powdered europium oxide (EuO) and erbium sulfide (ErS) were homogeneously mixed by mortar and pestle, and pressed into pellets. The pellets were sealed, however, in an evacuated tantalum crucible and heated at  $1750^\circ C.$  for approximately 8 hours and cooled down to room temperature within a 30 minute period. The reacted mixture formed a two-phase system and exhibited a paramagnetic Curie temperature ( $\theta$ ) of  $130^\circ K.$

#### Example 4

Similar procedures were followed as in Example 3 with respect to the europium oxide (EuO)-gadolinium sulfide (GdS) system. For example, finely-powdered europium oxide (EuO) and gadolinium sulfide (GdS) were formed in a homogeneous mixture of 85 percent-15 percent by mole and pressed into pellets. The pellets were sealed in an evacuated tantalum crucible and heated at  $1750^\circ C.$  for approximately 8 hours. The reacted mixture was then cooled to room temperature within a 30 minute period. The reacted mixture formed a two-phase system and exhibited a paramagnetic Curie temperature ( $\theta$ ) of  $130^\circ K.$

Because of the similar chemical properties of the remaining reactants (RS), it is clear that similar solid solutions of europium oxide (EuO) and any of the (RS) monosulfides will give corresponding increases in paramagnetic Curie temperature ( $\theta$ ).

While the invention has been particularly described with reference to preferred embodiments thereof, it will be understood by those skilled in the art that various changes in form and details may be made therein without departing from the spirit and scope of the invention.

What is claimed is:

1. A ferromagnetic material having the formula



where  $0.01 < x < 0.30$  and R is a rare earth element selected from the group consisting of lanthanum (La), praseodymium (Pr), neodymium (Nd), samarium (Sm), gadolinium (Gd), cerium (Ce), dysprosium (Dy), terbium (Tb), holmium (Ho), erbium (Er), thulium (Tm), and lutetium (Lu).

2. A ferromagnetic material having the formula



where  $0.01 < x < 0.30$ .

3. A ferromagnetic material having the formula



where  $0.01 < x < 0.30$ .

4. A ferromagnetic material having the formula



where  $0.01 < x < 0.30$ .

5. A ferromagnetic material having the formula



where  $0.01 < x < 0.30$ .

6. The method of forming a ferromagnetic material having the formula  $(\text{EuO})_{1-x}(\text{RS})_x$ , where  $0.01 < x < 0.30$  and (RS) is a monosulfide of a rare earth element selected from the group consisting of cerium (Ce), lanthanum (La), erbium (Er), and gadolinium (Gd), praseo-

dymium (Pr), neodymium (Nd), samarium (Sm), dysprosium (Dy), terbium (Tb), holmium (Ho), thulium (Tm), and lutetium (Lu) comprising the steps of mixing europium oxide (EuO) and said monosulfide, heating said mixture to react at least a portion of said mixture to form a solid solution of said europium oxide (EuO) and said monosulfide, and rapidly cooling said mixture to room temperature.

7. The method of claim 6 comprising the further step of cooling said mixture to room temperature within a 30 minute period.

8. The method of claim 6 comprising the further step of heating said mixture whereby a portion thereof enters into a liquid phase.

#### References Cited

##### UNITED STATES PATENTS

3,234,494 2/1966 Matthias ----- 252—62.51

##### OTHER REFERENCES

Didchenko et al.: "Some Electrical and Magnetic Properties of Rare Earth Monosulfides and Nitrides," J. Phys. Chem. Solids, vol. 24, 1963, pages 863—870.

25 TOBIAS E. LEVOW, Primary Examiner.

ROBERT D. EDMONDS, Examiner.